

July 2, 1946.

J. J. MISKEL

2,403,293

ANTICORROSION COMPOSITION

Filed June 5, 1943



INVENTOR  
*John Joseph Miskel*

BY  
*Harold A. Swanson*

ATTORNEY

## UNITED STATES PATENT OFFICE

2,403,293

## ANTICORROSION COMPOSITION

John Joseph Miskel, Brooklyn, N. Y., assignor to  
 National Oil Products Company, Harrison, N. J.,  
 a corporation of New Jersey

Application June 5, 1943, Serial No. 489,784

10 Claims. (Cl. 106—14)

**1**  
 This invention relates to temporary oily and greasy coatings for application to metallic objects to prevent the corrosion thereof, and more particularly to such compositions containing surface-active fatty amino compounds.

It is the practice in the metal-working industry to coat finished or semi-finished metallic components with oily or greasy compositions to preserve them from corrosion during subsequent working, storage or shipment. This practice is highly necessary, but entails a considerable inconvenience. For instance, when using oily compositions for this purpose, it is necessary to thoroughly dry the metallic objects to be treated before applying the corrosion-proofing coating thereto, since otherwise any water on the surface of the objects will be entrapped and will cause local corrosion. Since metallic objects are almost always pickled, phosphated, plated, blacked, anodized, etc., as a final step in the manufacture thereof, this necessity for careful drying occurs very frequently, and consumes a vast amount of time, equipment, space and labor in the metal working industries. Further, even though a metallic surface may be macroscopically dry, it frequently carries an absorbed surface film of moisture, which materially reduces the effectiveness of the various rust proofing compounds hitherto employed.

Accordingly, it is an object of this invention to provide oily corrosion-proofing compositions which may be applied to wet metallic objects, and which will displace the water on the surface thereof to provide a corrosion-proofing film directly in contact with the metal.

Another object is to provide corrosion-proofing compositions which will penetrate and displace the microscopic film of adsorbed moisture almost universally occurring on the surfaces of metallic objects so as to provide a more effective anti-corrosion film.

Another object is to provide rust proofing compositions of the types outlined above which will be cheaply and readily made from cheaply and readily procurable raw materials.

The foregoing and other objects are achieved in accordance with this invention by the incorporation into an oily composition designed for application to metallic surfaces for corrosion-proofing purposes of a small quantity of a higher

**2**  
 fatty amino compound. Such an amino compound will impart to the composition the property of displacing any moisture whether in the form of macroscopic water drops or in the form of an adsorbed vapor film on any metallic surface so as to form an oily coating in immediate molecular contact with the metallic surface and to prevent the corrosion thereof.

The oily or greasy bodies to which fatty amino compounds are added according to this invention may be substantially the same as those hitherto employed for corrosion proofing coatings, which usually consist of petroleum or fatty oils or mixtures of petroleum or fatty oils, usually with the petroleum oil, which is cheaper, in predominant proportion. Suitable petroleum oils are any naphthenic or paraffinic petroleum oils of sufficiently low volatility, noncorrosiveness and viscosity to be suitable metal-coating agents. Suitable fatty oils are the animal, marine and vegetable oils, and preferably the fatty acids derived therefrom. Examples of suitable fatty oil materials are sperm oil, cod oil, train oil, pilchard oil, lard oil, neat's-foot oil, olive oil, cottonseed oil, and the like; and fatty acid oils such as red oil, stearic acid, coconut fatty acids, fish oil fatty acids and the like. Likewise tall oil and naphthenic acids may be employed, since they possess properties generally similar to those of the fatty acids.

As fatty amino compounds to be incorporated into oily and greasy corrosion-proofing compositions according to this invention there may be employed any substances containing fatty chains of "surface active" length, i. e., having from about 10 to about 22 carbon atoms per molecule, and also containing one or more primary or secondary amino groups, such as the higher fatty amines and amido-amines. Examples of suitable fatty amines include dodecyl amine, lauryl amine, palmityl amine, stearyl amine, oleyl amine and the like. Instead of compounds containing amino groups directly attached to the fatty carbon chain, there may be employed compounds in which the amino groups are on organic groups attached by ether, ester or amide linkages to the fatty carbon chain, such compounds being represented, for instance, in the amido-amines on the order of oleyl monoamide of diethylene triamine, the stearyl monoamide of diethylene triamine, the oleyl

monoamide of ethylene diamine, dodecyl monoamide of diethylene triamine, etc. Particularly favorable results have been secured by the use of the oleyl monoamide of diethylene triamine. Instead of the pure compounds there may, of course, be employed mixtures containing one or more compounds coming within the qualifications above set forth, for instance, the fatty amines and fatty amido-amines derived from the natural oils, fats and waxes. Moreover, since the naphthenic acids and tall oil possess properties generally in line with those of the animal and vegetable fats and oils, the amines and amido-amines containing the high molecular radicles of these materials may likewise be employed. The amount of the fatty amino compound incorporated into the only compositions of this invention may be very small, amounts on the order of  $\frac{1}{4}\%$  to 1%, based on the total oily composition, being sufficient to secure results in accordance with this invention. Greater quantities may be added, as dictated by particular requirements and economic considerations.

The corrosion-preventive oily and greasy compositions of this invention may be applied to metal components and other objects in the same manner as has been the practice with similar compositions in the past, i. e. by dipping, spraying, mopping, brushing, etc. However, in contrast to the practice heretofore, it is unnecessary to insure absolute dryness of the surfaces to be treated; in fact the compositions of this invention will actually displace macroscopic accumulations of water occurring on metal surfaces and will effectively form a corrosion proofing film over the metal despite the former presence of the water. This property will be seen to result in a great saving of time and labor in the corrosion proofing of metallic objects, since it will be unnecessary to dry such objects after phosphating, pickling, blacking, anodizing, etc., treatments; the object to be treated may simply be rinsed in water, drained free of the rinsed water insofar as this will spontaneously run off and then, without further draining or inspection, immersed in the anticorrosion compositions of this invention. Somewhat less spectacularly, the compositions of this invention have been found to form corrosion preventing films upon metallic surfaces which are dry to visual inspection, which films are of superior effectiveness as compared to similar compositions heretofore prepared. This is no doubt due to the fact that metallic objects generally contain an adsorbed film of moisture which the compositions of the present invention are capable of displacing but which the compositions of the prior practice simply entrap.

Following are examples of compositions according to this invention, and of the use thereof, all parts given being by weight.

#### Example I

In this and in succeeding examples, accelerated corrosion tests were conducted upon steel panels treated with compositions according to this invention and also, for purposes of comparison, upon steel panels treated by other methods. The tests were conducted upon treated 4" x 6" panels of 18 gage SAE-1015CF steel. The panels were mounted upon a turntable which carried them alternately into a chamber maintained at 70° F. and 25% humidity and into a chamber maintained at 160-170° F. and 100% humidity, 65

this cycle being completed every 3 minutes. Condensation on the panels occurred in the moist chamber, and reevaporation in the dry chamber, at each cycle, thus providing unusually severe corrosive conditions. The surface of each panel was examined periodically and the rust spots on the entire surface of both faces of that panel were counted and taken as a measure of the corrosion of that panel. Obviously the less the number of rust spots found at any given time upon a given test panel, the more effective the protection of that panel must have been. The corrosive conditions encountered in this test may be taken to represent exposure to normal conditions of transportation and storage of 10 to 100 times the actual time of exposure in the apparatus.

The following rust-proofing coatings were prepared.

*Composition A.*—Not in accordance with this invention, merely for purposes of comparison.

|                                 | Parts |
|---------------------------------|-------|
| 25 Chromium soap of wool grease | 20    |
| V. M. & P. naphtha              | 80    |
| <hr/>                           |       |
| 100                             |       |

*Composition B.*—In accordance with this invention.

|                                     | Parts |
|-------------------------------------|-------|
| Tall oil                            | 8½    |
| Oleic monoamide of ethylene diamine | 1½    |
| Mineral oil                         | 90    |
| <hr/>                               |       |
| 100                                 |       |

*Composition C.*—In accordance with this invention.

|                                     | Parts |
|-------------------------------------|-------|
| Tall oil                            | 8½    |
| Oleic monoamide of ethylene diamine | 1½    |
| Chromium soap of wool grease        | 18    |
| V. M. & P. naphtha                  | 72    |
| <hr/>                               |       |
| 100                                 |       |

1. A set of cleaned steel panels were wet with water and then directly immersed while still wet in Composition A above. The panels were left in the composition for 10 minutes and then withdrawn and allowed to drain for 60 hours. They were then subjected to the accelerated corrosion test set forth above. The average results of this corrosion test are recorded graphically in curve 1 of the drawing and also in the table at the end of Example IV hereinbelow (item under "Example I, paragraph 1"). It will be noted that the protection afforded was only partial, since a considerable number of rust spots developed almost immediately.

2. A set of cleaned steel panels were carefully dried and immersed in Composition A for 10 minutes. The panels were removed, allowed to drain for 60 hours and then subjected to the accelerated corrosion test. The average results are recorded graphically in curve 2 of the drawing and in the table hereinbelow ("Example I, paragraph 2"). It will be noted that fair resistance to corrosion was provided by this treatment.

3. A set of cleaned steel panels were wet with water and dipped in Composition B. Thereafter 75 they were removed from the Composition B and

## 5

immersed for 10 minutes in Composition A. Thereafter the panels were removed from Composition A, allowed to drain for 60 hours and then subjected to the accelerated corrosion test, the average results of which are graphically recorded in curve 3 of the drawing and in the table hereinbelow ("Example I, paragraph 3"). It will be noted that the use of Composition B, which contains fatty amido-amine (oleic mono-amine of ethylene diamine) in accordance with this invention, resulted in superior performance over the panels treated as described in the immediate preceding paragraph 2 although the panels of paragraph 2 were absolutely dry as far as could be determined by visual inspection, whereas the panels treated in accordance with this paragraph were initially wet with water.

4. A set of cleaned steel panels were preliminarily wet with water and were immersed while still wet in Composition C for 10 minutes. Thereafter the panels were removed, drained for 60 hours and subjected to the accelerated corrosion test, the average results of which are recorded graphically in curve 4 of the drawing and also in the table hereinbelow ("Example I, paragraph 4"). (The long and elaborate soaking and draining were merely for the purpose of insuring uniform test conditions, and are not necessary in the usual practice of this invention.) It will be seen that this composition gave outstanding performance, with only very gradual onset of any corrosion whatsoever and very slight final corrosion, notwithstanding the fact that the panels upon which this treatment was carried out were initially wet with water.

35

## EXAMPLE II

## TREATMENTS COMBINED WITH CAUSTIC BLACKENING

| Composition D                          |  | Parts |
|----------------------------------------|--|-------|
| Coumarone-indene resin                 |  | 11.8  |
| Lead soap of wool grease               |  | 3.2   |
| "Vistac" <sup>1</sup> polyisobutylenes |  | 1.0   |
| Tall oil                               |  | 3.4   |
| Oleyl monoamide of diethylene triamine |  | .6    |
| V. M. & P. naphtha                     |  | 80.0  |
|                                        |  | 100.0 |

40 45 50 55 60

(<sup>1</sup> "Vistac" is a trade name belonging to Advance Solvents and Chemical Corporation designating mixed polymers of butylene and isobutylene having a molecular weight between 1100 and 2400.)

This example was carried out upon steel panels which had been preliminarily cleaned and treated with a caustic blackening agent in order to show the cumulative effect of compositions according to this invention upon such blackened panels, which possess a certain amount of corrosion resistance aside from any oil treatment. A number of steel panels were given a caustic blackening treatment in a commercial solution ("Ebonol" manufactured by the Enthone Company, New Haven, Connecticut). This treatment was carried out by immersing the panels for 40 minutes in the boiling "Ebonol" solution, the boiling point of which was maintained at 290° F. by periodic additions of water. The panels were then rinsed 3 times in cold water.

1. A set of panels treated with "Ebonol" as just described were immediately subjected to the accelerated corrosion test without further treat-

## 6

ment. As will be seen from the table hereinbelow ("Example II, paragraph 1"), the panels were completely rusted at the end of the test.

2. A set of panels treated with "Ebonol" as above set forth were dried in sawdust and then immersed in Composition C of Example I for 10 minutes, drained for 24 hours and thereafter subjected to the accelerated corrosion test. As will be seen from the table hereinafter ("Example II, paragraph 2") only a slight amount of corrosion occurred within 500 hours, at the end of which time the test was discontinued.

3. A set of panels still wet from the final rinsing of the "Ebonol" treatment were directly immersed in Composition C for 10 minutes, removed, drained for 24 hours and subjected to the accelerated corrosion test. Only slight corrosion resulted over the 500-hour period in which the test was conducted, see the table "Example II, paragraph 3".

4. A set of panels which had been subjected to the "Ebonol" treatment were dried in sawdust and immersed in Composition D for 10 minutes, removed, drained for 24 hours and subjected to the accelerated corrosion test. Only slight corrosion resulted (table, "Example II, paragraph 4").

5. A set of panels still wet from the final rinse in the "Ebonol" treatment were immersed in Composition D for 10 minutes, removed, drained for 24 hours and subjected to the accelerated corrosion test. Only minor corrosion resulted (table, "Example II, paragraph 3").

## EXAMPLE III

## TREATMENTS COMBINED WITH PHOSPHATING

The procedure of Example II was precisely repeated, with the exception that the steel plates, instead of being treated with "Ebonol," were phosphated at 203° F. for 60 minutes in a "Parkerizing" solution, which is a commercial phosphating composition manufactured by The Parker Rust-Proof Company. The results of these tests are included in the table following Example IV, the items "Example III, paragraph 1" to "Example III, paragraph 5." It will be seen that in each case the treatments of this invention greatly enhanced the recognized rust-proofing qualities of the "Parkerizing" treatment.

## EXAMPLE IV

## TREATMENTS COMBINED WITH PHOSPHATING

The procedure of Examples II and III was precisely repeated, with the exception that the steel panels, instead of being treated with "Ebonol" or "Parkerizing solution," were phosphated at 200° F. for five minutes in a "Bonderizing" solution, which is a commercial composition manufactured by the Parker Rust-Proof Company. The results of these tests are included in the table following this example, the items "Example IV, paragraph 1" to "Example IV, paragraph 5." It will be seen that in each case the treatments of this invention greatly enhanced the recognized rust-proofing qualities of the "Bonderizing" treatment. It will be appreciated, in connection with this and the preceding two examples, that the ability to oil metal objects while still wet from rinsing after the "Ebonol," "Parkerizing" and "Bonderizing" treatments makes possible a great saving in time and labor.

75

## Accelerated corrosion tests

| Example No. | Paragraph No. | Pretreatment of panels | Condition of panels treated | Oil treatment compositions | Average number of rust spots on panels |        |        |        |         |         |
|-------------|---------------|------------------------|-----------------------------|----------------------------|----------------------------------------|--------|--------|--------|---------|---------|
|             |               |                        |                             |                            | 24 hr.                                 | 36 hr. | 60 hr. | 84 hr. | 108 hr. | 100 hr. |
| I           | 1 (curve 1)   | None                   | Wet                         | A                          | 55                                     | 30     | Rusted |        |         |         |
| I           | 2 (curve 2)   | do                     | Dry                         | A                          | 8                                      | 14     | 22     | 22     | 22      |         |
| I           | 3 (curve 3)   | do                     | Wet                         | B, then A                  | 4                                      | 10     | 12     | 22     | 22      |         |
| I           | 4 (curve 4)   | do                     | do                          | C                          | 0                                      | 1      | 3      | 4      | 4       |         |
| II          | 1             | "Ebonol"               | do                          | No oil treatment           | 1                                      | 4      | 10     | 11     | 75      |         |
| II          | 2             | do                     | Wet                         | C                          | 0                                      | 0      | 0      | 0      | 0       |         |
| II          | 3             | do                     | Dry                         | C                          | 0                                      | 0      | 0      | 0      | 0       |         |
| II          | 4             | do                     | Wet                         | D                          | 0                                      | 0      | 0      | 0      | 0       |         |
| II          | 5             | do                     | Dry                         | D                          | 0                                      | 0      | 0      | 0      | 0       |         |
| III         | 1             | "Parkersized"          | do                          | No oil treatment           | Rusted                                 | 0      | 0      | 0      | 0       | 0       |
| III         | 2             | do                     | Wet                         | C                          | 0                                      | 0      | 0      | 0      | 0       |         |
| III         | 3             | do                     | Dry                         | C                          | 0                                      | 0      | 0      | 0      | 0       |         |
| III         | 4             | do                     | Wet                         | D                          | 0                                      | 0      | 0      | 0      | 0       |         |
| III         | 5             | do                     | Dry                         | D                          | 0                                      | 0      | 0      | 0      | 0       |         |
| IV          | 1             | "Bonderized"           | do                          | No oil treatment           | Rusted                                 | 0      | 0      | 0      | 0       | 0       |
| IV          | 2             | do                     | Wet                         | C                          | 0                                      | 0      | 0      | 0      | 0       |         |
| IV          | 3             | do                     | Dry                         | C                          | 0                                      | 0      | 0      | 0      | 0       |         |
| IV          | 4             | do                     | Wet                         | D                          | 0                                      | 0      | 0      | 0      | 0       |         |
| IV          | 5             | do                     | Dry                         | D                          | 0                                      | 0      | 0      | 1      | 2       | 18      |

Example V  
SLUSHING COMPOUND BASE

|                                    |       |       |    |
|------------------------------------|-------|-------|----|
| High melting point petrolatum      | Parts | 52.0  | 25 |
| Tall oil                           |       | 14.5  |    |
| Scale wax                          |       | 6.0   |    |
| Wool grease                        |       | 6.0   |    |
| Oleyl amide of diethylene triamine |       | 1.5   |    |
| Petroleum solvent                  |       | 20.0  | 30 |
|                                    |       | 100.0 |    |

The foregoing was a very satisfactory slushing compound base which was capable of further dilution with solvents for final application to various metallic surfaces such as steel, brass, copper, aluminum etc. When so applied, rust and/or corrosion was substantially completely prevented on the treated surfaces.

Example VI  
HOT-MELT APPLICATION SLUSHING COMPOUND

|                                      |       |       |    |
|--------------------------------------|-------|-------|----|
| High melting point petrolatum        | Parts | 55.0  | 45 |
| Low melting point petrolatum         |       | 25.0  |    |
| Wax (M. P. 170° F.)                  |       | 10.0  |    |
| Vistac <sup>2</sup> polyisobutylenes |       | 4.0   |    |
| Red oil                              |       | 3.4   | 50 |
| Mahogany soaps                       |       | 2.0   |    |
| Octadecyl amine                      |       | .6    |    |
|                                      |       | 100.0 |    |

<sup>2</sup> Trade name of Advance Solvents & Chemical Co.

The above composition meets the Army and Navy Air Craft Specification ANC-52 type 2, grade A, adapted for application to external surfaces in molten form by dipping, mopping or brushing. It was found to be highly effective in preventing corrosion of all metallic surfaces under very severe conditions of exposure.

EXAMPLE VII  
SLUSHING COMPOUND

|                                    |       |       |    |
|------------------------------------|-------|-------|----|
| Heavy mineral oil                  | Parts | 71.0  | 65 |
| Low melting point petrolatum       |       | 25.0  |    |
| Tall oil                           |       | 3.4   | 70 |
| Oleyl amide of diethylene triamine |       | .6    |    |
|                                    |       | 100.0 |    |

The foregoing composition was a very satisfactory slushing compound and was found capable

of protecting various metallic surfaces against corrosion for extended periods of time.

From the foregoing specification it will be seen that compositions according to this invention provide greatly improved protection for metallic surfaces even when compared to compositions of the prior art when applied to dry surfaces. Moreover, compositions of this invention may be applied to wet metallic surfaces, thus providing a great saving of time and labor over the practice heretofore, which necessitated the careful drying of all surfaces to be protected. Furthermore, the compositions of this invention may be very cheaply made, since they require the addition of only a very small amount of any of a number of fatty amino compounds, which compounds are themselves cheaply and readily procurable.

I therefore claim:

- An anticorrosion coating composition for metals comprising an oily material containing a minor proportion, in an amount to function as an anticorrosive agent, of a fatty amido-amine containing fatty chains of from 10-22 carbon atoms.
- An anticorrosion coating composition for metals comprising chiefly mineral oil and a minor proportion, in an amount to function as an anticorrosive agent, of a fatty amido-amine containing fatty chains of from 10-12 carbon atoms.
- An anticorrosion coating composition for metals comprising chiefly mineral oil and a fatty oil with a minor proportion, in an amount to function as an anticorrosive agent, of a fatty amido-amine containing fatty chains of from 10-22 carbon atoms.
- An anticorrosion coating composition for metals comprising chiefly mineral oil and tall oil with a minor proportion, in an amount to function as an anticorrosive agent, of a fatty amido-amine containing fatty chains of from 10-22 carbon atoms.
- An anticorrosion coating composition for metals comprising chiefly mineral oil and a fatty oil with a minor proportion, in an amount to function as an anticorrosive agent, of the oleic acid monoamide of diethylene triamine.
- An anticorrosion coating composition for metals comprising chiefly mineral oil and tall oil and a minor proportion, in an amount to function as an anticorrosive agent, of the oleic acid monoamide of diethylene triamine.
- A method of preserving wet metallic surfaces from corrosion which comprises coating said

surfaces while still wet with a composition comprising an oily material containing a minor proportion, in an amount to function as an anticorrosive agent, of a fatty amido-amine containing fatty chains of from 10-22 carbon atoms.

8. A method of preserving wet metallic surfaces from corrosion which comprises coating said surfaces while still wet with a composition comprising chiefly mineral oil and a fatty oil together with a minor proportion, in an amount to function as an anticorrosive agent, of a fatty amido-amine containing fatty chains of from 10-22 carbon atoms.

9. A method of preserving wet metallic surfaces from corrosion which comprises coating said 15

surfaces while still wet with a composition comprising chiefly mineral oil and tall oil together with a minor proportion, in an amount to function as an anticorrosive agent, of a fatty amido-amine containing fatty chains of from 10-22 carbon atoms.

10. A method of preserving wet metallic surfaces from corrosion which comprises coating said surfaces while still wet with a composition comprising chiefly mineral oil and tall oil together with a minor proportion, in an amount to function as an anticorrosive agent, of the oleic acid monoamide of diethylene triamine.

JOHN J. MISKEL.

**Certificate of Correction**

Patent No. 2,403,293.

July 2, 1946.

JOHN JOSEPH MISKEL

It is hereby certified that errors appear in the printed specification of the above numbered patent requiring correction as follows: Column 3, line 17, for "only" read *oily*; column 8, line 50, claim 2, for "10-12 carbon atoms" read *10-22 carbon atoms*; and that the said Letters Patent should be read with these corrections therein that the same may conform to the record of the case in the Patent Office.

Signed and sealed this 10th day of September, A. D. 1946.

[SEAL]

**LESLIE FRAZER,**  
*First Assistant Commissioner of Patents.*

surfaces while still wet with a composition comprising an oily material containing a minor proportion, in an amount to function as an anticorrosive agent, of a fatty amido-amine containing fatty chains of from 10-22 carbon atoms.

8. A method of preserving wet metallic surfaces from corrosion which comprises coating said surfaces while still wet with a composition comprising chiefly mineral oil and a fatty oil together with a minor proportion, in an amount to function as an anticorrosive agent, of a fatty amido-amine containing fatty chains of from 10-22 carbon atoms.

9. A method of preserving wet metallic surfaces from corrosion which comprises coating said 15

surfaces while still wet with a composition comprising chiefly mineral oil and tall oil together with a minor proportion, in an amount to function as an anticorrosive agent, of a fatty amido-amine containing fatty chains of from 10-22 carbon atoms.

10. A method of preserving wet metallic surfaces from corrosion which comprises coating said surfaces while still wet with a composition comprising chiefly mineral oil and tall oil together with a minor proportion, in an amount to function as an anticorrosive agent, of the oleic acid monoamide of diethylene triamine.

JOHN J. MISKEL.

**Certificate of Correction**

Patent No. 2,403,293.

July 2, 1946.

JOHN JOSEPH MISKEL

It is hereby certified that errors appear in the printed specification of the above numbered patent requiring correction as follows: Column 3, line 17, for "only" read *oily*; column 8, line 50, claim 2, for "10-12 carbon atoms" read *10-22 carbon atoms*; and that the said Letters Patent should be read with these corrections therein that the same may conform to the record of the case in the Patent Office.

Signed and sealed this 10th day of September, A. D. 1946.

[SEAL]

**LESLIE FRAZER,**  
*First Assistant Commissioner of Patents.*